

## UNITED STATES PATENT OFFICE

2,352,293

## PAPERMAKING

John C. Sherman, Attleboro, Mass., assignor to  
A. P. W. Paper Co., Inc., Albany, N. Y., a corpora-  
tion of New York

No Drawing. Application January 10, 1940,  
Serial No. 313,200

2 Claims. (Cl. 154—50)

This invention relates to an improved construction of such papers as are treated with suitable impregnants and piled together with or without reinforcements of twine or fibres, to constitute tough, water-resistant protective membranes as for the sheathing of buildings, the wrapping of goods, the lining of shipping cases and forms for cement-pouring in the construction of buildings. Other well-known applications are for agricultural uses as in the protection of crops and produce, and wherever structures or goods have to be protected from climatic exposure. Such papers are used upon freshly laid concrete or cement highway—"lanes" to ensure slow and suitable curing, and in the facing of excavations and the like.

Such papers are commonly formed of two sheets of kraft or other suitable paper adhered together with an intermediate film of asphalt or the like, or with pastes or glue suitably conditioned for the purpose.

That face of each sheet which is affected by the asphalt (hereinafter called the "inner" face) is combined with the inner face of its mated sheet through the adhesive quality of the asphalt (or the like) employed, the combining process usually being hastened and made effective by hot pressure.

In the production of such plied papers, it is customary to use for the two plies a sized paper, the sizing serving both to toughen the paper and to prevent the absorption of so much asphalt (e. g.) as would become objectionable through "bleeding" or thorough permeation of the paper with the impregnant to a point whereat the outer faces of the sheets would themselves become tacky, difficult to roll up and to handle.

The said impregnant is therefore not commonly used in amounts adequate to ensure the stout bonding together of the papers.

The adhesive film is commonly tenuous and discontinuous in spots, with resulting penetration of water or water-vapor into the interior of the plied material.

In many instances such papers, at the moment when their inner faces are to be pressed together, as above, receive between them a deposit of coarse open-meshed fabric, or a network or other system of textile cords or yarns as of jute or cotton, or of raw strands of natural vegetable

fibre simulating the result to be obtained with more organized textile inserts.

When such papers are so combined, with intermediate reenforcing material, the presence of such material still further militates against the firm and continuous bonding of the two sheets.

Especially when strands of some natural fibre are so used, as the intermediate re-enforcing element, such strands, being relatively incompressible and intractable in the application of them to the composite sheet, create along each such fibre a potential zone of deficient waterproofness. Such zones, each of thread-like fineness but high capillarity, readily accept vapor passed to them through the imperfectly coated sheets. Such vapor, condensed, remains and continues to reduce the effectiveness of the adhesive "bond," the fibres themselves reacting to this condition by being rapidly disintegrated.

20 To offset in part such objectionable effects, it has been proposed to add to such plied composites an intermediate film of a highly bibulous paper or other sheet, which said sheet is, before or during the final combining process, heavily 25 impregnated as with asphalt. When a three-ply construction is thus produced, a more effective barrier against water and/or vapor is provided. The bibulous sheet receives the textile material more or less within its soft and yielding structure, and the larger amount of asphalt used with it improves the general bonding effect, despite the reluctance of the sized outer sheets to accept a sufficient quota of asphalt.

However, the penetration of vapor through 35 these outer sheets is not thus prevented, and the textile materials and the bibulous film itself become moist; and, when a moist condition is prolonged or intermitted but interminably repeated, the deterioration of the material ensues, since, in a wet state, the elements of construction are deficient in strength.

However, the inclusion of this intermediate bibulous film has great utility, while dry, for these following reasons: (a) the film itself, after 45 impregnation, followed by the consolidating effect of that pressure which is used to compress the composite material, materially adds to the tear and tensile strengths of the composite; (b) the "bond" between the outer sheets is greatly 50 facilitated, so that the composite material in use

has less tendency to wrinkle, or to blister from atmospheric water and/or vapor; (c) the bibulous film makes with the reenforcing textile material so good a bond that the textile material is more adequately kept in place against the displacing influences of prolonged stress as when the material is nailed or battened to an exposed wall.

The asphalt, now having a material with which it can adhesively unite, resists the pulling effects of such use, which effects commonly result in a progressive displacement of the reinforcements.

Disadvantageous results occur, however, from the rapid deterioration of the bibulous film along with the outer plies from wetness, as, notwithstanding its partial protection from asphalt, it remains to a degree hydrophilic, a result which follows from its nature and the inability of the mill process described above to give it to an entirely effective waterproofness.

I have found it practicable to build up a bibulous film having unusually high Mullen and tensile strength when wet, as by suitable treatment with impregnants combined with tanning or other setting factors which conserve the original quality of the film to a marked degree when wet, without materially diminishing its acceptance of molten asphalt or other water-proofing saturant.

A composite material therefore, as produced under this invention, may have either of two final forms. (First) it may comprise two external sheets of the usual sized paper each of which has been treated on and in its inner face with asphalt, and an intermediate film of wet-strengthened paper-like material; all being bonded as by hot pressure. (Second) it may comprise two external sheets as above, treated as stated, a central wet-strengthened film as above, and—intermediate between said film and said sheets—it may have a deposit of textile material in woven, knitted, netted or more or less random formation, said deposit being made upon either one or both faces of said film.

There is a third form of construction one may make without departing from the scope of this invention, consisting in wet-strengthening both the intermediate bibulous film and either one or both of the external paper sheets, such sheets for external use to be given the wet-strengthening treatment before they are resin-sized in the conventional tub-sizing way.

Means for imparting to a thin, bibulous film of paper-making material a high degree of mechanical strength when wet are to some extent known today and may be used in carrying out this invention.

Among such means are the treatment of the said film, prior to its inclusion in the composite structure of my invention, with a bath of water containing appropriate mixtures of glue and a chemical such as formaldehyde which strengthens the glue against weakness from wetting; also, alternatively, one may use a bath of the fluid components of a synthetic resin, such as a resin described in U. S. Patent #2,111,698 of March 22, 1938, to Siefert and Stadler on the process of preparing hydrophobic cellulose "fibre"—whereby is meant each individualized fibre—provided sufficient resinous bath is used to affect the inter-fibrous voids in the sheet formed with such resinous content. Or a somewhat equivalent protection can be given by a bath of dextrin with its appropriate fixatives; or the requisite wet-strength may be obtained by the wet-strength-

ening of the pulp by above means in the beater or before it is converted into paper.

Any of these or other methods of immunizing a cellulosic fibre against the effects of wetness 5 may be used in my invention without departing from my invention.

Also, the bibulous film itself along with the paper sheets which form the outer plies of my structure, may be individually or together given 10 a wet-strength as by any of the above or other means.

Such treatment must be given to each individual ply—that is, to the bibulous film and to the paper sheets of the outer plies—if such treatment precedes the combining process whereby 15 the said film and the said sheets, along with whatever reenforcing strands or the like—if any are used, are combined.

This would be the usual practice in that instance where a non-aqueous cementitious binder 20 is used—such as asphalt—to combine the plied structure. But in other instances, wherein the binder is sufficiently hydrophylic, the wet-strengthening treatment of my central ply or of 25 all plies, may take place coincidently with the plying operation and subsequent drying processes.

To those skilled in the arts of sizing and otherwise impregnating cellulosic fibres and fibrous films and sheets, it will be obvious that all of the 30 above noted methods of wet-strengthening have as their common characteristic that they do not, if properly used, produce a sheet which is thereafter incapable of receiving either aqueous or non-aqueous impregnants and bonding or cementing agents, but that they serve to affect all adjacent individual fibres by a bond itself immune to destruction from wetness.

Thus, for example, if I apply to a bibulous 40 (so-called "water-leaf") film of reasonably uncompacted structure—(say of a density, according to the accepted scale of paper densities, of from 30 to 75) a treatment, as by tub-dipping or by "kissing-rolls," with glue and formaldehyde in water, and thereafter dry the film so treated, 45 it remains stout when wet, but is relatively unaffected so far as concerns its subsequent treatment with asphalt in a molten state or in a water-dispersed or "colloidal" or emulsified fluid form, or by other acceptable impregnants, such as starch, starch or dextrine with fixatives included, case-in glue, or any of the usual synthetic resins in their fluent form.

As an instance, I have treated a water-leaf 55 sheet of a mixed furnish of sulphite and ground-wood with a bath of glue and formaldehyde so prepared as to add to 100 grams-weight of said sheet, air dry, an added weight of impregnants of about 5% air dry, up to 10%, according to the 60 strength of the glue so used, and have thereafter noted the following tabulated characteristics:

|                                    | Mullen strength dry of original sheet | Mullen strength wet after soaking in water |
|------------------------------------|---------------------------------------|--------------------------------------------|
| 65                                 |                                       |                                            |
| Basis-weight of sheet, 32 lbs..... | 4                                     | 10                                         |

Air dry weight of impregnant, 3 lbs.....

70

This result is taken as typical; though in practice, to bring the sheets so tested within the scale-reading of my Mullen machine, I have had to insert into the Mullen machine four plies of the dry and four plies of the wet sheet for compari-

son; scale readings being for such tests: 16 points for the dry and 40 points for the wet sheets.

The period of preliminary immersion in water for the wet test was ten seconds, but I have found no material reduction of wet Mullen after prolonged water-soaking.

The absorptivity of the treated sheets for subsequent impregnation is broadly noted in a typical test as follows:

*Comparison of treated and untreated paper*

|                                                                   | Water absorbed<br>Grams |
|-------------------------------------------------------------------|-------------------------|
| 100 grams air dry water-leaf sheet before treatment               | 300                     |
| 105 grams of same stock (100 grams pulp<br>5 grams of impregnant) | 250                     |

Weight of absorbed water was figured by prolonged immersion of both types of sheet in water, then hanging up to dry until dripping substantially stopped, and then weighing.

It will be clear to those skilled in the art relative hereto, that, especially with the glue-formaldehyde treatment, I have set up within the gross structure of the paper a sort of synthetic resin.

The glue-formaldehyde mixture, after being dried in bulk, sets up as a horny material similar to the known resins.

But in the minimal amounts of such resin which I form as above and apply to paper, this formation of horn-like product is not materially effective to alter the ordinary characteristics of the paper.

Thus the "water-crawl" is not markedly affected, flexibility remains satisfactory, and the dry-strength of the sheet not materially changed since I have avoided subsequent subjection of the sheet to such heavy pressure as is usual in the sizing of ordinary paper.

This method of impregnation is commonly believed, as my tests confirm, to serve mostly as a means of attaching individual cellulose fibres or shreds of fibre to one another, while leaving the gross structure of the sheet not markedly affected adversely to subsequent impregnation.

The cementitious union of adjacent contacting fibres effected by the treatment does, however, serve, (as indicated by the tabulation above) to prevent the dislocation of such fibres when stressed in a water-soaked condition.

It is, therefore, evident that the film of paper treated for use in my invention does not revert to a wet-pulpous condition when subjected to seepage of water in the plied structures which I produce.

If, in the further application of my invention, it is desired to render all the plies, or the outer plies alone, or one of them, immune to injury

from wetness, the sheet for which such application is to be made should be run off without heavy sizing of the conventional saponified-resin type or the like.

5 It should be treated in its bibulous form with any of my stated impregnants, such as the glue-formaldehyde mixture, applied in a tub-sized system or by a "kissing" roll, to the necessary degree to immunize it to water.

10 Thereafter it may be tub-sized with the conventional sizings to give it stiffness, superficial water-resistance, and the familiar characteristics of a normally-sized sheet.

Such sizing, as resin-sizing, is not desired for 15 the central ply for which the highest possible residual absorptivity for impregnants such as asphalt is desired.

For the outer sheet or plies, often for uses 20 where exposure to the weather is an incident of use, the normal characteristics of a sheet for such exposure, as with a resin size, are desirable.

These outer sheets, especially the sheet for 25 exposure to weather as in sheathing or wall-covering paper, may indeed shrink away from whatever fastening means are used to hold them in place, and thus become cracked or ruptured either along the confining means or at some intermediate place.

In this case, the efficacy of my central ply, 30 treated as described, now becomes important as a means of protecting the plied material from final disintegration.

The central ply, with its coatings of asphalt 35 or other ply-cementing agency, is in itself effective to cement the outer sheet in place, despite localized lines of rupture, and in itself it resists the further development of weakness in the plied structure under wet conditions of use.

Having thus described my invention without 40 limitation to the specific steps enumerated or to the limited fields of application enumerated, I claim:

1. A composite paper comprising outer sheets 45 of Kraft paper, an intermediate film of bibulous wet-strengthened paper, said sheets being absorptive to asphalt, and asphalt films between said sheets and said film of bibulous wet-strengthened paper bonding them together.

2. A composite sheet comprising outer sheets 50 of Kraft paper, a centrally disposed sheet of bibulous wet-strengthened paper, a deposit of textile strands disposed upon the central sheet, said sheet and textile strands being absorptive to asphalt, and a film of asphalt between the adjacent 55 faces of the sheets and embedding the textile strands and bonding the sheets and strands together.

JOHN C. SHERMAN.